

Patented Sept. 4, 1923.

1,466,907

# UNITED STATES PATENT OFFICE.

LESTER KIRSCHBRAUN, OF CHICAGO, ILLINOIS, ASSIGNOR TO THE RAYBESTOS COMPANY, OF BRIDGEPORT, CONNECTICUT, A CORPORATION OF CONNECTICUT.

## FRICITION FACING AND PROCESS OF MAKING SAME.

No Drawing. Application filed August 16, 1920, Serial No. 404,012. Renewed February 13, 1922. Serial No. 536,343.

To all whom it may concern:

Be it known that I, LESTER KIRSCHBRAUN, a citizen of the United States, residing in the city of Chicago, county of Cook, and 5 State of Illinois, have invented certain new and useful Improvements in Friction Facings and Processes of Making Same, of which the following is a specification.

This invention relates to improvements in 10 friction facings and process of making same and refers more particularly to a friction element such as a clutch ring adapted for use in motor cars and the like.

The object of the invention is to provide 15 a friction facing made from relatively cheap incombustible fibre, as for example, short asbestos fibres, which facing is impregnated or saturated with a relatively cheap binder but which, nevertheless, has 20 the required coefficient of friction, Brinnell hardness and tensile strength.

The process may be carried out as follows: The friction facings, as for example, clutch rings, may be cut out of asbestos millboard 25 and calendered and dried in the usual way. These rings are then immersed in a saturating solution. This saturating solution consists of asphalt or asphaltic oil dissolved in phenol to which may be added a thinning 30 vehicle such as petroleum gas oil. It may not be necessary to use pure phenol as any of the coal tar distillates, containing tar acids of this nature, may answer the purpose. The percentages of the ingredients, of 35 course, may be varied, although a mixture of 80% Mexican asphalt, of less than 100 melting point, to 20% of phenol may be used. The proportions will vary with the nature of the materials used and the object sought to be obtained. The friction facings may be immersed in this saturating solution for a period of several hours or until they are thoroughly impregnated and then removed. The facings are then either immersed in a bath of formaldehyde or subjected to the action of formaldehyde vapors, which results in forming phenol resin in the ring.

It may be desirable in certain cases to subject the ring to a slight baking after the first saturating step referred to and before treatment with formaldehyde. The object of this baking is merely to remove excess volatile products in the facing and leave the

facing in prime condition for action by the 55 formaldehyde. After the formaldehyde treatment, the facings are placed in an oven and subjected to a baking operation at a sufficient highly temperature to thoroughly cure and harden the facing and this treatment is continued until the facing has a tensile strength in excess of 2,000 pounds to the square inch and a Brinnell hardness in excess of 15. The extent of the baking and the temperature used will, of course, vary with the character of the phenol or coal tar distillate used and also with the character of the asphalt. For example, if an oxidized asphalt or the air blown asphalts of commerce are used, it will tend to bake more 70 readily than where a relatively thin or liquid asphalt is employed which has not been oxidized. In any event, the baking operation should be continued until the asphalt becomes unaffected by heat and insoluble in the usual solvents for asphalt. The retained saturant in the finished facing will consist, in large, part, of the cheap asphaltic material with sufficient phenolic condensation products to insure the desired 75 strength and hardness.

The following modified method of carrying out the process may sometimes be advantageously employed. Instead of subjecting the saturated facing to the formaldehyde treatment, this step may be obviated by incorporating in the facing an oxidizing agent, as for example, lead oxide or lead 85 resinate.

I claim as my invention:

1. A process of making a friction facing consisting in forming a facing element from unwoven sheeted asbestos fibre, saturating said element in a solution of bituminous substance and phenol, removing the saturated 95 element and subjecting it to the action of formaldehyde and then baking or curing the saturated element to the desired strength and hardness.

2. A process of making a friction facing consisting in forming a facing element from unwoven sheeted asbestos fibre, saturating said element in a solution of bituminous substance and phenol, removing the saturated element and subjecting it to the action of formaldehyde and then baking or curing the saturated element to the desired strength 105 and hardness and continuing said baking

and curing until the element has a Brinnell hardness in excess of 15 and a tensile strength exceeding 2,000 pounds to the square inch.

5 3. A process of making a friction facing, consisting in forming a facing element from unwoven sheeted asbestos fibre, saturating

said element in a solution of bituminous substance and phenol, removing the saturated element and subjecting it to the action of <sup>10</sup> formaldehyde and curing the element to the desired strength and hardness.

LESTER KIRSCHBRAUN.